

May 13, 1930.

A. M. THOMSEN

1,758,896

MANUFACTURE OF PAPER PULP

Filed Aug. 1, 1927



INVENTOR.  
Alfred M. Thomsen  
BY  
Lounseid, Poltus & Ackett  
ATTORNEYS.

## UNITED STATES PATENT OFFICE

ALFRED M. THOMSEN, OF SAN FRANCISCO, CALIFORNIA

## MANUFACTURE OF PAPER PULP

Application filed August 1, 1927. Serial No. 209,791.

This invention relates to improvements in the manufacture of paper pulp; the improvements which I have effected deal in a general way with the use of alkali sulphides such as sodium sulphide, potassium sulphide or a mixture of both as a cooking liquor.

As used to-day in the processes known by the names of "sulphate" and "kraft," sodium sulphide is used in conjunction with caustic soda as the means of liberating the cellulose fiber from the encrusting materials. It is generally held that the principal agent in the progressive hydrolysis, destruction and solution of the encrusting substances is the caustic soda and that the sulphide only comes into play close to the end when the caustic soda is almost or entirely spent.

The present system of recovery includes evaporation, incineration, smelting, leaching and causticizing. This produces a peculiar mixture of sulphate, carbonate, hydrate and sulphide of soda, the cooking liquor before referred to, which gives the special results wanted in the sulphate and kraft processes. The loss of soda is made up by the addition of sodium sulphate.

In my process I rely entirely upon sodium or potassium sulphide to dissolve the encrusting substances which necessitates a radically new method for the regeneration of the alkali salts employed; in my process I employ in place of this series of operations, evaporation to a syrupy consistency, absorption in charcoal or briquetting with charcoal, destructive distillation with recovery of the volatile products, leaching of the resulting charcoal for the recovery of the alkali salts, and separation of the alkali carbonate produced in the process so as to preserve a strong sulphide solution. The loss of alkali is made up by the addition of sulphide.

The fiber produced by this process is very hard to bleach with chlorine or its derivatives, but it may be easily bleached by means of permanganate or more cheaply by means of a solution of alkali manganate with or without the aid of  $\text{CO}_2$ . My process is therefore, best considered under three aspects, namely, (a) the cooking of the pulp, (b) the

regeneration of the cooking liquor, (c) and the bleaching of the fiber.

The several steps of the invention are shown in the accompanying drawing which illustrates a diagrammatic flow sheet of the process.

(a) *Cooking*.—The solvent action of strong solutions of sulphide upon the encrusting matters is so much greater than upon the fiber that very varying woods or mixtures of woods and barks, or such materials as bamboo, grass, straw, sugar cane bagasse, cornstalks, etc., are readily resolved into pulp. It is not necessary to cook under pressure, as a sufficiently strong solution will do the work just as well under atmospheric conditions. I can, therefore, employ simple tanks with filter bottoms, with or without circulation of the cooking liquor, such as are generally used in cooking esperto. However, if weaker solutions are desired, tanks which permit cooking under pressure may be employed.

(b) *Regeneration*.—When a cook is finished, the pulp is washed free from liquor, and both cooking liquor and wash water evaporated to the consistency of syrup. This is now mixed with sufficient charcoal to stiffen it. It may be either briquetted or put in shallow trays, placed on proper metal cars and run into an oven as if it were cord wood. By means of heat the organic combinations with alkali are resolved into charcoal, volatile substances, and alkali salts. The volatile products are recovered, refined and marketed. The charcoal and alkali salts are separated by leaching out the alkali, which is present partly as carbonate, partly as sulphide. As the former is the less soluble salt, it is removable, partially at least, by fractional crystallization, and so prevented from accumulating to an undue extent. The loss of alkali is made up by the addition of sulphide. The charcoal is used in part to "stiffen" a succeeding charge, the rest is burnt, or marketed.

(c) *Bleaching*.—As produced by this process the fiber is of a blackish gray to brown color, very strong and free from encrusting matter. As stated before, it is very hard to

bleach it with chlorine or its derivatives but it yields easily to permanganate. I have found alkali manganates equally efficient. It is easily prepared by fusing manganese ore with caustic alkali, dissolving the melt in water and using the resulting green solution in place of permanganate. If  $\text{CO}_2$  or washed chimney gases be blown through simultaneously, the action is expedited. The spent liquor may be separated from the pulp, brought up to strength with fresh manganate and re-used. After a number of such repetitions it will become so strong in alkali that same may be profitably extracted. The pulp is subsequently cleaned by means of sulphur dioxide in the customary manner. Here, also, the process may be rendered cyclic and the dissolved manganese ultimately precipitated and recovered.

Having thus described my invention, what I claim and desire to secure by Letters Patent is:—

1. A process for liberating fiber obtained from a vegetable source from encrusting materials which consists in cooking the fiber in a solution of alkali sulphide only, washing the fiber, bleaching the fiber by subjecting it to a solution of alkali manganate, and simultaneously passing carbon dioxide gas through the solution.

2. A process for liberating fiber obtained from a vegetable source from encrusting materials which consists in cooking the fiber in a solution of alkali sulphide only, washing the fiber, bleaching the fiber by subjecting it to a solution of alkali manganate, and then cleaning the fiber by subjecting it to the action of sulphur dioxide.

3. A process for liberating fiber obtained from a vegetable source from encrusting materials which consists in cooking the fiber in a solution of alkali sulphide only, washing the fiber, bleaching the fiber by subjecting it to a solution of alkali manganate, simultaneously passing carbon dioxide gas through the solution, and then cleaning the fiber by subjecting it to the action of sulphur dioxide.

ALFRED M. THOMSEN.